

H. WITTEBORG.

METHOD OF AND APPARATUS FOR RECOVERING VOLATILE METALLIC VALUES IN THE FORM OF  
METALLIC OXIDS FROM MOLTEN SLAG.

APPLICATION FILED MAR. 6, 1917.

1,250,261.

Patented Dec. 18, 1917.

2 SHEETS—SHEET 1.



Inventor

Herman Witteborg.

By Wilkinson, Gunst & Mackay

his Attorneys.

H. WITTEBORG.

METHOD OF AND APPARATUS FOR RECOVERING VOLATILE METALLIC VALUES IN THE FORM OF  
METALLIC OXIDS FROM MOLTEN SLAG.

APPLICATION FILED MAR. 6, 1917.

1,250,261.

Patented Dec. 18, 1917.

2 SHEETS—SHEET 2.



Fig. 2.

Inventor

Herman Witteborg.

By Wilkinson, Ginstat & Mackay

His Attorneys

# UNITED STATES PATENT OFFICE.

HERMAN WITTEBORG, OF CALDWELL, IDAHO.

## METHOD OF AND APPARATUS FOR RECOVERING VOLATILE METALLIC VALUES, IN THE FORM OF METALLIC OXIDS, FROM MOLTEN SLAG.

1,250,261.

Specification of Letters Patent. Patented Dec. 18, 1917.

Application filed March 6, 1917. Serial No. 152,729.

To all whom it may concern:

Be it known that I, HERMAN WITTEBORG, a citizen of the United States, residing at Caldwell, in the county of Canyon and State 5 of Idaho, have invented certain new and useful Improvements in Methods of and Apparatus for Recovering Volatile Metallic Values, in the form of Metallic Oxids, from Molten Slag; and I do hereby declare the 10 following to be a full, clear, and exact description of the invention, such as will enable others skilled in the art to which it appertains to make and use the same.

This invention relates to the recovery of 15 volatile metallic values, in the form of metallic oxids, from molten slag.

For the sake of brevity, I shall simply employ the terms "zinc" and "zinc oxids", but it will be understood that I do not limit 20 myself in this regard, as the invention itself is susceptible for use with other volatilizable metals or metallic compounds.

It may be stated at the outset that my invention is not for a smelting process for 25 the direct recovery of metals from crushed ores or from broken up briquets of slag containing metallic values. Neither is it for the recovery of raw metals, as such, by the simple volatilization and condensation 30 of distilled vapors, nor even does it broadly reside in the recovery of metallic oxids by the oxidizing of the zinc vapors distilled out of molten slag by treating the same in an externally heated retort containing a 35 large quantity of the molten slag, whether taken from a blast furnace, or re-smelted after having been formed into briquets containing a suitable flux and reducing agent. Finally, the invention does not 40 specifically rely upon the step of reacting upon the slag, in the form of a molten bath, by the introduction of a suitable agent for releasing and driving out the metallic values, all of which steps may be broadly 45 disclosed in the prior art.

It is true that it is one of my aims to avoid the necessity of re-smelting lump, granulated or briquetted slag, and to this extent I do take the molten slag directly 50 from its source of production. Also, in extracting its metallic values by volatilization, prior to final oxidation, I preferably, though not necessarily, introduce any of

the well known re-acting or reducing agents, as may be found expedient in practice. 55

Taken as a whole, however, I attain the desired ends, by additionally treating the molten slag in a manner which is believed to be more efficient, in certain of its steps and features, to the methods heretofore employed, the primary object of my invention being to increase efficiency and output, and at a substantially reduced expense in point of economy of time, attention required and cost of operation, all of which are manifestly of major importance. 65

My invention, therefore, is not merely directed to the broad idea of recovering zinc oxids from the vapors of molten slag, but wholly resides in the novel method and the 70 combined arrangement and functioning of the elements of the apparatus hereinafter disclosed, the essential steps and features of which will be succinctly stated in the appended claims, when viewed in the light of 75 the following detailed description and accompanying drawings, forming a part of this application, in which drawings—

Figure 1, illustrates a practical systematic arrangement of elements for carrying out 80 the improved method, being a view in plan of my improved apparatus itself, with certain minor elements omitted.

Fig. 2, is a vertical sectional view through 85 a pair of communicating units, taken along the plane of the line 2—2 of Fig. 1, and showing the addition of a twyer nozzle and bottom container pan omitted from Fig. 1, and

Fig. 3, is a vertical sectional view taken 90 transversely through a slightly modified construction of a retort unit, illustrating the application of a jacketed cooling chamber for the bottom of the retort units, if desired, and also showing the twyer nozzles 95 on the opposite side of the retort to that shown in Fig. 2.

Referring first to the preferred arrangement of elements as shown in Fig. 1, the numeral 5 designates the lower part of a 100 blast furnace provided with a slag outlet 6 and a discharge spout 7, which is preferably in indirect communication with an inlet pipe or trough 8 discharging, through a suitable opening, into the first unit of my 105 improved system.

The discharge spout 7 of the blast furnace is preferably spaced from the inlet pipe 8 of the first unit, so as to permit of the interposition of a slag settling pot 9, 5 into which the spout 7 empties, and provided with a short lip or spout 10 at its upper peripheral edge, the said settling pot being suitably mounted on a wheeled carriage support, whereby it may be readily 10 withdrawn for dumping and replaced in position.

The numeral 11 designates generally the several retort units, hereinafter more specifically described, which may be provided 15 at their discharge ends with collection hoods 12 communicating through elbows or branch pipes 13 with a main conduit 14 for carrying off the volatilized metallic values, in the form of metallic oxids, to suitably located 20 collection receptacles not shown.

Referring now to Fig. 2, the units 11 are of substantially narrow and elongated structure, the walls of which are built up of fire brick, as shown, or of any other suitable 25 highly refractory material or elements.

The bottom walls 15 may be of level surface, over which flows a continuous stream of the molten slag, in the form of a shallow sheet or ribbon-like layer. The top wall 16 30 is preferably arched.

The front wall is apertured at its base to provide a slag outlet 17 discharging into a refractory spout 18, which in turn empties, through an inlet opening 19 in a side wall of 35 a retort, into the interior of the next adjacent unit of the series, the inlet opening 19 of the first unit receiving the pipe 8 and the spout 18 of the last unit discharging to waste, as clearly shown in Fig. 1.

The rear wall of each unit is provided 40 with a flame opening 20, through which is injected a naked flame, of great intensity and substantial force, generated from powdered coal or coke, gas or oil, or other form 45 of fuel. For convenient illustration, I have shown an oil burner 21, its fuel feed pipe being designated at 22 and a pressure air pipe at 23. Additional air, for obvious purposes may be drawn in through the space 50 between the burner nozzle and flame opening.

The top wall of each unit may also be provided with an opening 24 for the introduction of a flux or a reducing agent of any 55 suitable character, when expedient, and these openings may be maintained closed with suitable plugs as desired.

At the forward end of each unit, the top wall 16 is substantially apertured, as at 25, 60 or entirely omitted, over which open spaces are mounted the collecting hoods 12, previously referred to, the open bottoms of the hoods preferably projecting slightly beyond the side walls of the units, as indicated at 65 26 (Fig. 1) to provide substantial air inlets

to the hoods from the outer atmosphere, for assisting in the oxidation of the volatilized metallic values vaporized off of the shallow stream of the molten slag as it is superheated in passing through the units.

While the various inlets and outlets have been shown as described, it is obvious that the disposition of these details may be varied in a different arrangement of the several units, so long as the molten slag is caused to 75 flow through the superheating zones in a shallow stream against the surface of which is directed the hot flames and gases of combustion.

To provide for the further addition of air, 80 preferably intensely heated and under substantial pressure for purposes hereinafter appearing, I project a twyer nozzle 27, or a series of such nozzles, through either or both side walls of the retorts, to discharge adjacent the bottom walls 15, beneath or into the flowing shallow stream of molten slag, which latter is indicated at 28. The upper ends of these twyer nozzles 27 are connected with a pipe line 29, common to all of them, 85 and leading from the source of compressed air. It is not deemed necessary to illustrate this source of compressed air nor controlling valves for the twyer nozzles, as the location of such elements are obvious, and these features have also been omitted from the illustrative plan view of Fig. 1, as being of 90 obvious disposition.

As previously stated, the body of each retort unit 11 is built up of suitable refractory 100 bricks or molded sections, and when assembled the walls are securely tied together by any suitable metallic skeleton frame work, or even a closed metallic sheathing if desired.

In Fig. 2 a preferred arrangement is shown, wherein the bottom of each unit is snugly seated in a pan or trough element 30, of boiler plate or sheet iron or their equivalent, the side walls of which may extend a 110 substantial distance upwardly along the side walls of the unit, providing a substantial base container support. Metallic bars 31 may also be disposed longitudinally of the top side wall surfaces, and the whole binding structure tied securely together by means of vertical metallic bars 32, appropriately apertured at their ends to receive the cross-tie bolt rods 33, extending transversely above the top of the unit and the bottom of the 115 container pan 30.

In Fig. 3, the twyer nozzle 27 is shown as projecting through the side wall opposite to that shown in Fig. 2, as the twyer nozzles may obviously enter from either or both 125 sides as desired, and other than this, provision is also made in this view for a jacked chamber 34 to contain a suitable non-conductor of heat, or circulating cooling 120 water.

The principles of the invention might be well carried out with apparatus other than described, but for the purpose of economy of space and other reasons, the arrangement of 5 a series of units at angles to each other has been found peculiarly fitted for the best results.

The actual dimensions of the units are not material, within fair limits, and they are 10 suitably mounted at a slight incline from their inlet ends to their outlet ends, with their discharge outlets sufficiently restricted, so that the flow of the molten slag, through the several units after the first one, is in the 15 nature of a sluggish stream or layer, the depth of which is comparatively shallow, say three inches or less, for it will be recognized the thinner the layer, the more quickly will it be superheated and volatilized as the 20 naked flame and hot gases play directly thereon.

From the foregoing description it is believed that the invention will be fairly apparent, but the functioning of the apparatus 25 and the steps of the process may be more specifically defined by the following statement.

A charge of hot molten slag is tapped from the blast or other furnace 5 into the 30 slag settling pot 9, through the spout 7, and overflowing into the spout 10, passes through the inlet pipe 8 into the first unit, substantially filling the latter to a line below its burner. At the same time, the first unit begins to empty, through its discharge spout 35 18, into the next unit, and so on throughout the remainder of the series as set forth.

The amount of slag drawn from an ordinary blast furnace at each tap is usually 40 from 1000 to 1500 pounds, and each tap is from ten to fifteen minutes apart. From computation, it will take from ten to fifteen minutes, approximately, for the first unit to empty, and a similar amount of time for 45 the slag to flow through each successive unit, so that by the time that the blast furnace is ready for another tap, the first unit will be ready to receive the charge, without interfering with the operation of the remaining 50 units.

As the slag flows from the first unit, its depth is gradually diminished therein, becoming hotter and hotter, and as it flows through each successive unit, in a shallow 55 stream, it is superheated to the high state of volatilization by the direct action of the blast of flame thereon, which action also ruffles its surface to agitate the mass and present a constantly changing surface to the direct action 60 of the flame and heated gases. The flowing slag is also agitated to a minor degree in its passage from unit to unit.

This treatment, of causing the blast flame and hot gases to directly impinge upon the 65 surface of a layer of slow flowing slag, has

alone been found sufficient to so highly superheat the slag as to readily extract the zinc vapors therefrom, but naturally the addition of a flux such as limestone, or a reducing agent such as coke, greatly facilitates and 70 accelerates the action.

The zinc vapors arising are then substantially aerated by the incoming fresh air through the spaced openings 26, causing them to become rapidly oxidized, whereupon 75 they are conveyed off to the filter bags or other collection receptacles, not shown, through the hoods and connections with the main conduit 14, through which a suctional force may be created by any suitable means 80 not necessary to illustrate.

Where the shallow stream of slag is constantly agitated to present a continuously changing new surface, it is manifest that the intense flame and hot gases playing thereon 85 is caused to more intimately contact with the molecular particles throughout the mass, thus greatly accelerating vaporization with a maximum recovery of the zinc values.

By the employment of the air twyer nozzles 27, I have found that this agitation can be effectively governed to meet varying conditions, while affording additional air for oxidizing purposes, the air under pressure being forced into or below the slag, and 95 bubbling therethrough provides a forceful but more or less smooth agitation. If this compressed air is highly super-heated it will not tend to reduce the temperature of the slag, which necessarily must be maintained 100 at an extremely high temperature to vaporize its zinc values.

While I have thus fully disclosed my improved method and an apparatus successfully carrying out the steps thereof, it will 105 be understood that I do not limit myself to the exact details set forth, excepting as come within the purview of the ensuing claims and a reasonable construction of the scope thereof contemplating a fair range of equivalents.

What I do claim as new and patentable is:—

1. The method of recovering volatile metallic values from molten slag, which includes the steps of causing the molten slag, containing a suitable reducing agent, to flow, in a comparatively shallow layer, through an inclosed superheating zone; directing a sufficiently intense naked flame and its hot 115 gases, into positive intimate contact with the shallow layer of flowing slag, to cause the vaporization of the metallic values to be recovered; oxidizing the metallic vapors arising therefrom; and finally collecting the 120 oxidized vapors in the form of metallic oxids, substantially as described.

2. The method of recovering volatile metallic values from molten slag, which includes the steps of causing the molten slag, 130

containing a suitable reducing agent, to flow, in a comparatively shallow layer, through an inclosed superheating zone; causing the agitation of said flowing shallow layer of slag while directing a sufficiently intense naked flame and its hot gases, into positive contact therewith, to cause the vaporization of the metallic values to be recovered; oxidizing the metallic vapors arising therefrom; and finally collecting the oxidized vapors in the form of metallic oxids, substantially as described.

3. The method of recovering volatile metallic values from molten slag, which includes the steps of causing the molten slag, containing a suitable reducing agent, to flow, in a comparatively shallow layer, through an inclosed superheating zone; forcing air through said flowing slag to agitate the same; directing a sufficiently intense naked flame and its hot gases, into positive contact substantially with the molecular particles of said shallow layer of agitated flowing slag, to cause the vaporization of the metallic values to be recovered; oxidizing the metallic vapors arising therefrom; and finally collecting the oxidized vapors in the form of metallic oxids, substantially as described.

4. The method of recovering volatile metallic values from molten slag, which includes the steps of causing the molten slag, containing a suitable flux and reducing agent, to flow, in comparatively shallow layers, through a series of substantially closed communicating superheating retorts; causing the vaporization of the metallic values to be recovered by directing sufficiently intense blasts of naked flames and their hot gases into positive contact with the shallow layers of flowing slag; oxidizing the metallic vapors arising therefrom; and finally collecting the oxidized vapors in the form of metallic oxids from each superheated retort unit, substantially as described.

5. In apparatus for recovering volatile metallic values from molten slag, an elongated substantially closed superheating retort, having an inlet and an outlet for the molten slag and an outlet for oxidized vapors therefrom, and said retort being mounted and functioning to continuously flow a suitable charge of the molten slag therethrough in a comparatively shallow layer, in combination with means for directing a sufficiently intense blast of naked flame and its hot gases, into positive intimate contact with said flowing shallow layer of slag, to cause the vaporization of its metallic values to be recovered; means providing for the aeration of the metallic vapors, arising from said superheated slag, to oxidize the same; and means in communication with said oxidized vapor outlet for collecting the resulting oxidized vapors in the form of metallic oxids, substantially as described.

6. In apparatus for recovering volatile metallic values from molten slag, an elongated substantially closed superheating retort, having an inlet and an outlet for the molten slag and an outlet for metallic vapors arising therefrom and adapted to be oxidized, said retort being mounted and functioning to continuously flow a suitable charge of the molten slag therethrough in a comparatively shallow layer, in combination with means for injecting air currents through the body of said flowing shallow layer of slag to thoroughly agitate the same; means for applying heat to said agitated flowing shallow layer of slag of sufficient intensity to vaporize off its metallic values to be recovered; and means, in communication with said oxidized vapor outlet, for collecting the resulting metallic vapors in the form of metallic oxids, substantially as described.

7. In apparatus for recovering volatile metallic values from molten slag, the combination of a series of suitable elongated communicating superheating retort units, each having a slag inlet and outlet, and mounted and functioning to flow a suitable charge of the molten slag therethrough in comparatively shallow layers; a feed unit for said series adapted to receive a charge of the molten slag; flame openings through said units, disposed above the flow of slag therein; means for directing sufficiently intense blasts of naked flame and hot gases, through said flame openings into positive contact with the flowing shallow layers of slag, to cause the vaporization of the metallic values to be recovered; means providing for the aeration of the metallic vapors arising from said superheated flowing slag, to oxidize said vapors; an outlet for said recovered values; and means, in communication with said last named outlet, for collecting said oxidized vapors in the form of metallic oxids, substantially as described.

8. In apparatus for recovering volatile metallic values from molten slag, the combination of a communicating series of suitable retort units, each having a slag inlet and outlet, and mounted and functioning to flow a suitable charge of the molten slag therethrough in comparatively shallow layers; a feed unit for said series adapted to receive a charge of the molten slag; twyer nozzles, communicating with a source of compressed air, and discharging into said units below the line of flow of slag therein, for agitating said flowing slag; flame openings through said units, disposed above the flow of slag therein; means for directing sufficiently intense blasts of naked flame, though said flame openings into positive contact with the flowing shallow agitated layers of slag, to cause the vaporization of the metallic values to be recovered, said arising metallic vapors being oxidized by aeration; an outlet for the

recovered oxidized values; and means in communication with said last named outlet for collecting said recovered values in the form of metallic oxids, substantially as described.

9. In apparatus for recovering volatile metallic values from molten slag, the combination of a communicating series of suitable retort units, constructed, mounted and functioning substantially as described to cause a suitable charge of the molten slag to flow therethrough in comparatively shallow layers; burner openings discharging into said units above said flowing shallow layers of
- 10 slag; burners for said openings, functioning as described; an outlet in each of said units for the exit of the vapors arising from the superheated slag; hoods covering said outlets and providing openings for the admission of air to said metallic vapors to oxidize same; branch pipes leading from said hoods; and a suitable conduit, common to all of said branch pipes, for conveying off said oxidized vapors in the form of metallic oxids, substantially as described. 20 25

In testimony whereof, I affix my signature.

HERMAN WITTEBORG.